

Oct. 20, 1936.

W. H. MASON

2,058,334

CORRUGATED VEGETABLE-FIBER BOARD AND THE PROCESS OF MAKING SAME

Original Filed June 30, 1933 3 Sheets-Sheet 1



INVENTOR

WILLIAM H. MASON

BY

Dyke and Chaines  
ATTORNEYS

Oct. 20, 1936.

W. H. MASON

2,058,334

CORRUGATED VEGETABLE-FIBER BOARD AND THE PROCESS OF MAKING SAME

Original Filed June 30, 1933. 3 Sheets-Sheet 2



INVENTOR  
WILLIAM H. MASON  
BY  
*Dyke and Schaines*  
ATTORNEY

Oct. 20, 1936.

W. H. MASON

2,058,334

CORRUGATED VEGETABLE-FIBER BOARD AND THE PROCESS OF MAKING SAME

Original Filed June 30, 1933 3 Sheets-Sheet 3



INVENTOR

WILLIAM H. MASON

BY

Dyke and Schaines  
ATTORNEY

## UNITED STATES PATENT OFFICE

2,058,334

CORRUGATED VEGETABLE-FIBER BOARD  
AND THE PROCESS OF MAKING SAMEWilliam H. Mason, Laurel, Miss., assignor to  
Masonite Corporation, Laurel, Miss., a cor-  
poration of DelawareOriginal application June 30, 1933, Serial No.  
678,401. Divided and this application June  
29, 1934, Serial No. 732,954

7 Claims. (Cl. 154—33)

My invention relates to the making of corrugated vegetable-fiber board, and has for its principal object the provision of a process for converting flat sheets of vegetable-fiber board into sheets with permanent corrugations therein. Another object consists in the method of combining the corrugated board with flat boards for the making of rigid, girder-like products. Other objects are obvious or appear in connection with the following description of preferred embodiments.

In the accompanying drawings forming a part of this specification:

Figure 1 is a part end view and part transverse sectional view of one form of apparatus adapted for carrying out my invention;

Fig. 2 is a part plan view and part horizontal sectional view thereof, the sectional parts being taken substantially on the broken line 2—2 of Fig. 1;

Fig. 3 is a longitudinal sectional view taken substantially on the line 3—3 of Fig. 1;

Fig. 4 is a detail sectional view of actuating mechanism including toggles and hydraulic cylinders;

Fig. 5 is a schematic view of pipe connections and valving for controlling the admission of fluid to the hydraulic cylinders;

Figs. 6, 7 and 8 are diagrammatical sectional views to illustrate stages in the pressing operation.

Fig. 9 is a perspective view of a piece of the completed corrugated board; and

Fig. 10 is a cross sectional view of a built-up board, with stiffness and rigidity imparted thereto by use of corrugated board, and with facings of flat sheet board.

The apparatus shown is described and claimed in copending application Serial No. 678,401, filed June 30th, 1933, of which the present application is a division, and constitutes a simple form of hot pressing apparatus adapted for carrying out the present invention, having a framework 10 with cross beams 12 for fixedly supporting the bed of the corrugating hot press, which in the form shown consists of a series of hollow cylinders or pipes 16 arranged in parallel, and made of diameter and spacings dependent on the corrugation height and transverse spacings desired for the board, and which for a board of  $\frac{1}{8}$ " thickness 50 may desirably be in the neighborhood of 1 inch height of corrugation and 5 inch spacings between centers.

The movable press members also preferably consist of cylinders or pipes 18, located centrally over the openings 16 between the press-bed pipes

18, and mounted to have forcible movement toward and away from the bed pipes 16, as for example, individually carried by means of several pairs of toggle arms 20—22, which arms are pivoted at their respective ends to the pipes 18 and 5 to thrust beams 24 of the machine frame 10.

Actuation of the toggle arms and pipe 18 carried thereby may be by link members 26, common to all the toggles attached to each length of pipe, connecting rod 28, piston rod 30 and piston 32 of 10 hydraulic cylinders 34, which are rigidly supported, preferably in an end section 36 of the machine frame 10.

The movement of pipes 18 is confined to movement to and away from the pipes 16, and they are 15 restrained from lateral and endwise movement relative thereto. Such confinement may be secured by any suitable means, such as by providing each pipe 18 with vertical studs or standards 38 that work in openings or passages 40 20 provided between guide bars 42, 44 fastened in place in the machine frame as indicated at 46, and also between guide blocks 48 connecting the guide bars 42, 44. Such means or equivalent is shown at one end of the movable pipes 18 only, 25 but may be duplicated at each end of the pipes, if desired. The movable pipes 18 are further guided by being received in the recesses 16 between the fixed pipes 16.

The heating fluid, as steam, that is supplied to 30 the press pipes 16, 18 may be supplied to the fixed press-bed pipes 16 by the rigid pipe 52, and to the movable pipes 18 by the flexible piping 54, or hinged steam piping may be used, and preferably valved connections 56—58 are 35 provided for permitting a return circulation of the heating fluid, or same may be draw-off cocks for permitting escape of condensed steam.

In operation, the flat blank sheet 60 of vegetable-fiber that is to be corrugated, (having been 40 previously wet and otherwise prepared for treatment in manner hereinafter described), is inserted in place between the bed pipes 16 and the movable pipes 18, the latter having been raised to permit such insertion. The central press cylinder or pipe 18a is then forcibly depressed as by admission of oil or other fluid under pressure at 62 to the central one, 34a, of the hydraulic cylinders 34, this being accomplished, for example, by opening supply cock 62a, for this purpose, together with respectively closing and opening the discharge cocks 64 and 66 for such cylinder. The supply cock 62a, as well as the other like supply cocks for the other cylinders to be referred to, 45 after being opened, are left open during the 50 55

pressing operation so that the pressure is maintained and followed up during drying.

The movable pipes or cylinders 18b-18b, adjacent to the central pipe 18a and on each side thereof, are then forcibly depressed, as by supplying actuating fluid to the hydraulic pressure cylinders by means of supply cock 62b, which, as shown in Fig. 5, communicates with the two corresponding cylinders 34b, 34b. Extra width of material needed to make the curved section is thus supplied from each side inwardly while the center of the sheet is rigidly clamped.

This operation progresses continuously, from the central portion of the sheet being pressed toward each edge thereof, as by cock 62c being opened to supply actuating fluid to the cylinders 34c, 34c, thereby depressing press pipes 18c, 18c, and so on seriatim, press cylinder 34d, 34d being next operated so that pipes 18d, 18d are depressed, and finally the outer pair 34e, 34e.

Figure 6 shows the central press pipe or cylinder 18a depressed. Figure 7 shows same remaining depressed and with the adjacent press cylinders 18b, 18b depressed, and Figure 8 shows how this progressive pressing operation proceeds, the next adjacent pair of press pipes 18c, 18c being also depressed. It will be understood that series-operated valves, capable of rapid automatic actuation, can be used instead of the manual valves, which are illustrated and described for affording a simple disclosure and clear understanding of the invention and how it may be carried out.

The open character of the press platens consisting of the bed pipe 16 and movable press pipes 18 favors the rapid drying of the initially wet blank being operated on, the steam formed escaping freely through the board without the restraint that would be encountered with solid continuous platens. When the corrugated board is dry, the corrugated sheet, which is of substantially the original length, but of somewhat reduced overall width, is released by raising all the movable pipes 18 together, as by means of opening cocks to a supply inlet, 70, which may be common to all the cylinders 34 of the series, outlet valves 66 having been closed, outlet valves 64 opened, and supply valves 62 closed. This elevates the movable press cylinders or pipes 18, and the finished board can be removed.

The steps as above described can be followed with materials of various kinds having sufficient plasticity when wet and becoming rigid upon being dried out.

The preferred blanks to be used, however, are flat sheets of the hard, stiff, dense and strong composition board of my Patent No. 1,663,505, made from the wood or woody constituents of fibrous vegetable material, such as so-called soft wood or hard wood of trees, or of vegetable growths of various kinds, including bamboo, cane and other wood-forming grasses, and the like, reduced to fiber in a manner to retain sufficient of the non-cellulose constituents of the fiber to make it self-bonding; and a wet-lap of the fiber, preferably having about 2% of waterproofing petrolatum size incorporated, dried under heat and consolidating pressure, followed up as shrinkage proceeds, and with a wire screen in place between the wet-lap and a press platen. Such boards of specific gravity about one, or more than one, are well adapted for use with my invention.

To get best results and greatest freedom from breakage along the lines of corrugation and

least tendency to revert from corrugated state toward original flat state upon repeated wetting and drying of the corrugated board when exposed to the elements, as when used for roofing, such sheets, prior to being corrugated, are preferably given treatment, wholly or in part, as follows: The flat sheets to be corrugated are "tempered", as by incorporating with the fiber or impregnating the pressed sheet with about 2% to 5% by weight of siccative oil, as tung oil or linseed oil or mixtures thereof, and baked, as for a period of about 5 to 6 hours at about 300° F. This treatment gives a notable increase in the strength of the board when wet as well as when dry, and materially reduces the water absorption.

Further siccative oil is applied to the surface, preferably the wire-mesh surface of the sheet that is later to be corrugated, and the sheet heated for a short time, say about an hour, so that the oil will be retained in subsequent treatment.

The sheet is now submerged in water until it has taken up about 10 to 15% of water, which may require in the neighborhood of 24 hours. The water may be heated, or the sheet transferred to hot water to raise its temperature prior to insertion of the sheet into the corrugating press.

The wet sheet is then introduced into the corrugating press, and pressed and dried therein as already described. With steam in the pipes constituting the press platens at 70# per square inch, sheets  $\frac{1}{8}$ " thick are dried in about 20 minutes, the openwork construction of the spaced pipes permitting ready escape of the moisture.

The corrugated board that comes from the corrugating press is preferably now retempered as by submerging in a bath of siccative oil until about 2 to 5% by weight of oil has been absorbed, and removing and baking for about 5-6 hours at a temperature in the neighborhood of 300° F. Preferably, not over 5% of siccative oil is used in any tempering step or operation, since the strength curve falls off upon use of more oil than this, as for example, use of enough oil to produce saturation, and the baking period has to be excessively prolonged. With sheets treated in the manner described, the fibers are apparently locked in the corrugated position, for the corrugations are retained even under severe conditions of alternate wetting and drying out in use.

The corrugated sheet can be used in various ways similarly to sheets of corrugated iron, with the advantage that it does not readily transmit heat, needs no coating, and is free from rust and from corrosion, as when used in chemical plant construction, or exposed to salt air near the sea coast, and the like; by suitably modifying the corrugation spacing and height, the corrugated sheets can be cut into roofing tiles and the like, and high utility and good architectural effects obtained at low expense. With use of the corrugated board, I am enabled to make strong and stiff structural panels, to be used for walls and partitions of buildings, table tops and other places where a stiff panel is required, by planing the apices of the corrugations off flat to give a broad gluing surface as indicated at 88, Fig. 10, and gluing flat surface plates 82, 84 of vegetable-fiber board, tempered or untempered, thereto with waterproof glue or equivalent cementitious material, indicated at 86.

I claim:

1. Process of making corrugated hard vegetable-fiber board which comprises hot pressing corrugations into a wet sheet thereof progressively along openly spaced lines from the median line toward both edges thereof, and continuing the application of heat and pressure until substantially completely dry.
2. Process of making hard, corrugated board of vegetable-fiber which comprises forming vegetable fiber containing sufficient non-cellulose material to be self-bonding into a hard board by simultaneous application of consolidating heat and pressure, tempering same by incorporating about 2 to 5% of siccative oil material and baking at a temperature in the neighborhood of 300° F. for a period of several hours, wetting the tempered board, and drying it from wet state in a heated corrugating press, and re-tempering in substantially the same way as before.
3. Process of making hard, corrugated board of vegetable-fiber containing sufficient non-cellulose constituents to be self-bonding comprising forming same into a hard board by simultaneous application of consolidating heat and pressure until dry, wetting the board so produced, hot pressing the wet sheet progressively along openly spaced lines at each side and continuing the application of heat and pressure until substantially completely dry.
4. Process according to the preceding claim together with tempering the corrugated board by incorporating about 2 to 5% of siccative oil and baking at a temperature in the neighborhood of 300° F. for a period of several hours.
5. Stiff girder-like products comprising corrugated, hard vegetable-fiber board of specific gravity one or more than one and having flat surfaces of material width at the apices of the corrugations, and similar but flat surfacing boards cemented to the corrugated board along the flattened parts of the lines of corrugation.
6. Process of making corrugated hard vegetable-fiber boards which comprises applying heat and pressure to a wet blank of such material on one side along openly spaced apart lines and applying heat and pressure to the other side of the blank along openly spaced apart lines staggered in relation to the first set, and retaining the blank under pressure until substantially dried.
7. Process of making corrugated hard vegetable-fiber boards which comprises applying heat and pressure to a wet blank of such material on one side along openly spaced apart lines and applying heat and pressure to the other side of the blank along openly spaced apart lines staggered in relation to the first set.

WILLIAM H. MASON. 30